

## UNITED STATES PATENT OFFICE

GEORGE HOLLAND ELLIS, OF SONDON, NEAR DERBY, ENGLAND, ASSIGNOR TO  
CELANESE CORPORATION OF AMERICA, A CORPORATION OF DELAWARE

## TREATMENT OF MATERIALS MADE WITH OR CONTAINING CELLULOSE DERIVATIVES

No Drawing. Application filed March 25, 1927, Serial No. 178,504, and in Great Britain October 23, 1926.

This invention relates to the loading of 5 yarns or threads or woven, knitted, or other textile fabrics or other materials made of or containing artificial filaments or fibres of cellulose acetate or other organic acid esters of cellulose, for example, cellulose formate, propionate or butyrate, or cellulose ethers, for example, methyl, ethyl or benzyl cellulose, or the corresponding condensation 10 products of cellulose and glycols or other polyhydric alcohols, all of which are hereinafter referred to as organic substitution products of cellulose. The invention also relates to ribbons, films or similar products 15 made of the aforesaid organic substitution derivatives of cellulose.

It has been found that particularly good loadings are obtainable if the loading metals be employed at least in part in the form 20 of their thiocyanates.

Accordingly the present invention comprises a process for loading materials made of or containing organic substitution derivatives of cellulose and particularly cellulose 25 acetate, in which the goods are treated with a loading metal solution which contains the loading metal or metals at least partly in the form of thiocyanates.

The goods loaded according to the present 30 invention present considerable advantages over unloaded goods. Thus for example there is a reduction of the tendency of woven fabrics to "slip", of circular knitted fabrics to "ladder" and of warp knitted fabrics to "split", an increase in the fullness or volume of the yarns, threads or fabrics resulting in improved "handle" or feel and in economy of the material used to produce a given result, for example in a woven fabric 35 less ends and picks per inch will be needed to produce a given result than with unloaded materials; and the resistance to various agencies such as heat in ironing or finishing or aqueous treatments at high temperatures 45 is increased.

It is further found that the characteristic property, possessed by cellulose acetate in particular, of absorbing basic dyestuffs and dispersed insoluble dyestuffs is not deleteriously affected by this process. In fact

in some cases the rate of absorption is increased.

The loading metal may be fixed on the goods by treating them before or after the treatment with the loading metal solution 55 with a suitable precipitant for the loading metal. Thus for example the treatment with the loading metal solution may be preceded or followed by the application of a solution of tannic acid, a phosphate or silicate 60 or it may even be followed by a simple washing with water, preferably water containing some lime or other alkali in solution.

The proportions and concentrations of ingredients, and duration and temperature of 65 treatment may be varied widely according to the amount of loading required. Thus for instance cellulose acetate may be caused to absorb from very small proportions such as 1% of total loading to higher proportions 70 of say 100% or over.

The following examples are given by way of illustration, it being understood that they 75 are in no way limitative.

## Example 1

The weighting bath is prepared as follows:—

Concentrated aqueous solutions of stannic chloride and of ammonium thiocyanate are 80 mixed and made up with water so as to contain 280 grams of stannic chloride ( $\text{SnCl}_4 \cdot 5\text{H}_2\text{O}$ ) and 243 grams of ammonium thiocyanate per litre. These quantities are approximately those required to yield the 85 salt  $\text{Sn}(\text{CNS})_4$ .

Previously scoured cellulose acetate fabric is entered into the loading bath at about 20° C., and steeped for 1 hour with occasional turning. It is then lifted, drained well and 90 washed, first in two baths of cold water and then in two baths of water at 45° C. until quite free from soluble salts. The goods are next entered into a bath at 40° C. containing 12% of sodium dihydrogen phosphate, 95 worked for half an hour, lifted, rinsed and soaped for 20 minutes in a bath containing 2½ grams per litre of olive oil soap at 50° C. The goods are then rinsed and may be dried or otherwise treated as desired. 100

By this treatment the goods are weighted to approximately 20%. Heavier weightings may be obtained by a repetition of the process.

*Example 2*

Previously scoured cellulose acetate fabric is entered into a bath at 20° C. containing 280 grams of stannic chloride ( $\text{Sn Cl}_4 \cdot 5\text{H}_2\text{O}$ ) and 182 grams of ammonium thiocyanate per litre of liquor. These proportions represent approximately those necessary to obtain the salt  $\text{Sn Cl}(\text{CNS})_2$ . After steeping for 1 hour with occasional turning, the goods are lifted, drained, washed and further treated as described in Example 1. The goods are thus given a 20-25% weighting.

*Example 3*

A weighting bath is made up so as to contain 280 grams of stannic chloride ( $\text{Sn Cl}_4 \cdot 5\text{H}_2\text{O}$ ) and 121 grams of ammonium thiocyanate per litre of liquor, the proportions being approximately the proportions to form the salt  $\text{Sn Cl}_2(\text{CNS})_2$ . Previously scoured cellulose acetate fabric is then entered into the bath at about 20° C. and steeped for 1 hour with occasionally turning. The goods are lifted, drained well and washed twice in cold water and twice in water at 45° C. until the wash water is quite free from chlorine and thiocyanate. They are then treated for half an hour at about 40° C. in a 12% disodium hydrogen phosphate solution which has been rendered neutral to phenolphthalein by addition of a concentrated solution of ammonium chloride. The goods are now soaped for 20 minutes in a bath containing 2½ grams per litre of olive oil soap, rinsed well in soft water and dried or otherwise treated as desired. By this method the goods are given a weighting of 20-25%, the lustre being well preserved.

Alternatively in a more continuous process, the dry previously scoured goods may be passed through the weighting liquor in a suitable machine and squeezed so that they retain about their own weight of liquor, and allowed to stand for about 3 hours. The goods are then washed off and the treatment repeated, the goods being finally given a phosphate treatment. This process also gives a 20-25% weighting. For heavier weightings the number of treatments in the tin bath is increased until the desired increase is obtained.

Though in the above examples the thiocyanate has been employed in certain definite molecular proportions with respect to the tin, the invention is not limited to such proportions or of course to tin as loading metal. Further the proportion of thiocyanate may be increased so as to be in excess of that which is chemically equivalent to the whole

of the loading metal. Thus for instance in the case of tin it may be in excess of that necessary to yield the salt  $\text{Sn}(\text{CNS})_4$ . Further it will be understood that the loading metal thiocyanates may either be prepared <sup>70</sup> in situ in the baths as described in the above examples or they may be prepared prior to addition to the loading baths.

The process of the present invention may be applied to goods composed wholly of <sup>75</sup> cellulose acetate or other of the aforementioned organic substitution derivatives of cellulose, or to mixed goods, for example mixed fabrics containing yarns of wool, cotton, natural silk, artificial silk of the cellulose type, etc. or containing yarns composed of artificial filaments of cellulose acetate or other of the aforesaid organic substitution derivatives of cellulose doubled or associated with natural fibres, artificial silks of the cellulose type etc. <sup>85</sup>

What I claim and desire to secure by Letters Patent is:—

1. Process for loading materials comprising an organic substitution derivative of cellulose, comprising treating the materials with a loading metal solution containing loading metal at least partly in the form of thiocyanate. <sup>90</sup>

2. Process for loading materials comprising an organic substitution derivative of cellulose, comprising treating the materials with a loading metal solution containing loading metal at least partly in the form of thiocyanate and with a precipitant for the <sup>100</sup> loading metal. <sup>95</sup>

3. Process for loading materials comprising an organic substitution derivative of cellulose, comprising treating the materials with a solution containing tin at least partly in the form of thiocyanate. <sup>105</sup>

4. Process for loading materials comprising an organic substitution derivative of cellulose, comprising treating the materials with a solution containing tin at least partly in the form of thiocyanate and with a precipitant for tin. <sup>110</sup>

5. Process for loading materials comprising an organic substitution derivative of cellulose, comprising treating the materials with a solution containing tin at least partly in the form of thiocyanate and with a solution of a phosphate. <sup>115</sup>

6. Process for loading materials comprising cellulose acetate, comprising treating the materials with a loading metal solution containing loading metal at least partly in the form of thiocyanate. <sup>120</sup>

7. Process for loading materials comprising cellulose acetate, comprising treating the materials with a loading metal solution containing loading metal at least partly in the form of thiocyanate and with a precipitant for the loading metal. <sup>125</sup>

8. Process for loading materials comprising

<sup>130</sup>

ing cellulose acetate, comprising treating the materials with a solution containing tin at least partly in the form of thiocyanate.

9. Process for loading materials comprising cellulose acetate, comprising treating the materials with a solution containing tin at least partly in the form the thiocyanate and with a precipitant for tin.

10. Process for loading materials comprising cellulose acetate, comprising treating the materials with a solution containing tin at least partly in the form of thiocyanate and with a solution of a phosphate.

11. Process for loading materials comprising cellulose acetate, comprising treating the materials with a loading metal solution containing loading metal wholly in the form of thiocyanate.

12. Process for loading materials comprising cellulose acetate, comprising treating the materials with a loading metal solution containing loading metal wholly in the form of thiocyanate and with a precipitant for the loading metal.

13. Process for loading materials comprising cellulose acetate, comprising treating the materials with a solution containing tin wholly in the form of thiocyanate, washing and subsequently treating with a solution of a phosphate.

In testimony whereof I have hereunto subscribed my name.

GEORGE HOLLAND ELLIS.